# EUROPEAN PATENT SPECIFICATION

(11) **EP 0 356 246 B1**
(45) Date of publication and mention of the grant of the patent: **16.02.1994**
(21) Application number: 89308637.1
(22) Date of filing: 24.08.1989
(51) Int. Cl.: G03G 5/14, G03G 5/05

(54) **Photoreceptor**
Photorezeptor
Photorécepteur

(30) Priority: 25.08.1988 JP 211536/88
(43) Date of publication of application: 28.02.1990
(73) Proprietor: KONICA CORPORATION, Tokyo 160 (JP)
(72) Inventor: Takei, Yoshiaki, Hachioji-shi Tokyo 192 (JP); Sakai, Eiichi, Hachioji-shi Tokyo 192 (JP); Ichino, Tadasu, Hachioji-shi Tokyo 192 (JP); Matuura, Katumi, Hachioji-shi Tokyo 192 (JP)
(74) Representative: Wood, Anthony Charles

(56) References cited:
- US-A- 4 637 971
- PATENT ABSTRACTS OF JAPAN vol. 9, no. 129 (P-361)(1852) 05 June 1985, & JP-A-60 12551 (HITACHI) 22 January 1985,

## Description

### BACKGROUND OF THE INVENTION

The present invention relates to a photoreceptor such as one to be used in electrophotography.

In electrophotographic copying by the Carlson process, an electric charge layer is deposited on the surface of a photoreceptor and after exposure to form a latent electrostatic image, it is developed by a toner and the resulting visible image is transferred and fixed to a receiving sheet such as paper. Subsequently, the toner is removed from the surface of the photoreceptor and any residual charges are neutralized to erase the electrostatic image completely and condition the photoreceptor for another cycle, thereby enabling its cyclic use for a prolonged period.

For successful operation of electrophotography, the photoreceptor must satisfy various requirements not only in terms of electrophotographic characteristics such as good chargeability and sensitivity plus small dark decay but also in terms of physical properties such as long run length and high resistance to wear and moisture during cyclic use, as well as in terms of resistance to environmental conditions such as ozone generated upon corona discharging and ultraviolet radiation emitted during exposure.

Electrophotographic photoreceptors that have been commonly used in the art are inorganic products having a photosensitive layer that is based on inorganic photoconductive materials such as selenium, zinc oxide and cadmium sulfide. The use of various organic photoconductive materials as the effective component of light-sensitive layers in electrophotographic photoreceptors has been the subject of active research and development efforts in the recent years. For example, an organic photoreceptor having a light-sensitive layer containing poly-N-vinylcarbazole and 2,4,7-trinitro-9-fluorenone has been described in JP-B-50-10496 (the term "JP-B" as used hereunder means an "examined Japanese patent publication"). However, this photoreceptor is not completely satisfactory in terms of sensitivity and durability. In order to overcome this problem, attempts have been made to develop an organic photoreceptor of high sensitivity and durability by composing the light-sensitive layer of two different materials, one being responsible for carrier generation and the other for carrier transport. Electrophotographic photoreceptors of this "functionally separated type" provide for a great latitude in the selection of appropriate materials that exhibit the intended functions, and this enables photoreceptors having desired characteristics to be prepared fairly easily.

The organic electrophotographic photoreceptors described above have the advantage that the light-sensitive layer can be formed by coating techniques, so not only can they be manufactured at low cost without causing environmental pollution but they can also be fabricated in various forms including sheet. On the other hand, conventional organic electrophotographic photoreceptors have had the following problems that demand solution.
(1) The light-sensitive layer is formed of a low-molecular weight organic compound dispersed in a high-molecular weight organic binder resin, so that the mechanical strength of the layer is not high enough to prevent the photoreceptor's surface from being damaged or wearing by abrasion with the developing blade or some other phenomena that will occur during cyclic use of the photoreceptor.
(2) The photoreceptor is principally to be used as a negatively chargeable type and as shown in JP-A-60-247647 (the term "JP-A" as used hereunder means an "unexamined published Japanese patent application"), it is composed of a base that is overlaid with a thin carrier generation layer which in turn is overlaid with a comparatively thick carrier transport layer. When it is to be used as a negatively chargeable type, the photoreceptor has a large carrier (hole) mobility and permits the use of hole transporting materials, which is a definite advantage in such aspects as photosensitivity. In contrast, electron transporting materials available today very rarely have desirable characteristics or they are unsuitable for practical use because of their potential carcinogenic or teratogenic nature.
   A problem with the negatively chargeable photoreceptor is that negative corona discharging will generate an undesirably larger volume of ozone into the operating atmosphere during negative charging with a charging device than in the case of positive corona discharge, with consequent deterioration of the environmental condition. This causes either adsorption of ionic species onto the surface of the photoreceptor or deterioration of the material in its surface and the resulting decrease in potential during cyclic use will lead to various undesired phenomena such as increased residual potential, lowered sensitivity and deteriorated image quality, thereby reducing the service life of the photoreceptor.
(3) Electrophotographic copiers are to be used under various conditions for an extended period and are often placed under hot and humid conditions. It is therefore necessary to develop a practical photoreceptor that has high resistance to the environment.

US-A-4 637 971 discloses a photoreceptor which uses a polycarbonate resin having one of the formulas (I) and (II) described hereinafter. The document describes a photoreceptor which has good charging performance, repeatability and copy running life while avoiding the disadvantages of toner film build up and the like. The photoreceptor does not have good resistance to environmental factors such as ozone, heat and moisture.

JP-A-60 12551 discloses a photoreceptor in which the charge transport layer is composed of two or more constituent layers and in which the weight ratio of the content of the charge transport material to the binder in a constituent layer which is closer to the electroconductive base is higher than the weight ratio of the content of the charge transport material to the binder in a constituent layer which is more remote from the base. The purported object of the photoreceptor described in this document is to provide improved durability. However the photoreceptor does not possess satisfactory performance in hot and humid environments.

### SUMMARY OF THE INVENTION

An object, therefore, of the present invention is to provide a photoreceptor that has a high mechanical strength and good charging potential and sensitivity characteristics, that will not experience a substantial increase in residual potential, and that exhibits high resistance to the environment including hot and humid conditions.

According to the invention there is provided a photoreceptor having an electroconductive base, a carrier generation layer formed thereon, and carrier transport layer overlaid on the carrier generation layer and containing a carrier transport material and a binder material; the carrier transport layer comprising at least two constituent layers, so that the weight ratio of the carrier transport material to the binder material in a continuous layer which is closer to the electroconductive base is higher than the weight ratio of the carrier transport material in a constituent layer which is more remote from the electroconductive base, and a polycarbonate having as the principal recurring unit a structural unit represented by the following general formula (I) and/or a structural unit represented by the following general formula (II):
(where R¹ and R² each is a hydrogen atom, a substituted or unsubstituted aliphatic group, a substituted or unsubstituted carbocyclic group, or a substituted or unsubstituted aromatic group, provided that at least one of R¹ and R² is a "bulky" group; and R³, R⁴, R⁵, R⁶, R⁷, R⁸, R⁹ and R¹⁰ each is a hydrogen atom, a halogen atom, a substituted or unsubstituted aliphatic group, or a substituted or unsubstituted carbocyclic group);
(where R³, R⁴, R⁵, R⁶, R⁷, R⁸, R⁹ and R¹⁰ each is same as defined above; Z is the atomic group necessary to form a substituted or unsubstituted carbon ring or a substituted or unsubstituted heterocyclic ring).

### BRIEF DESCRIPTION OF THE DRAWINGS

Figs. 1 - 4 are partial cross sections showing different constructions of the electrophotographic photoreceptor of the present invention; and
Fig. 5 is a table showing the electrophotographic characteristics of the photoreceptor samples prepared in Examples 1 - 8 and Comparative Examples 1 - 6.

One of the major features of the photoreceptor of the present invention is that the carrier transport layer is divided into two or more constituent layers having different concentrations of carrier transport material. A constituent layer which is closer to said electroconductive base has a higher concentration of carrier transport material so that photocarriers generated in the carrier generation layer will be injected efficiently into the carrier transport layer. On the other hand, a constituent layer which is more remote from said electroconductive base has a lower concentration of carrier transport material, so that the reduced use of the carrier transport material having a low molecular weight will contribute to a corresponding increase in the mechanical strength of the carrier transport layer.

Another important feature of the present invention is that a polycarbonate having a structural unit represented by the general formula (I) and/or the general formula (II) as the principal recurring unit is incorporated as a binder in a constituent layer of said carrier transport layer which is the remotest from the electroconductive base. Polycarbonates having a structural unit represented by the general formula (I) and/or the general formula (II) as the principal recurring unit have high mechanical strength, good resistance to scratch and wear, long run length and desired charging performance. In particular, such polycarbonates have a hard surface while providing a reasonable degree of lubricity. They also have a high degree of transparency and insulating property and are highly miscible with the carrier transport material. In the polycarbonate, R¹ and R² at least one of which is "bulky" are bound to the central carbon atom of the bisphenol A portion or a ring is formed of Z around said carbon atom, so that said R¹ and/or R² or Z effectively prevents the molecular chain of the polycarbonate to be oriented in a certain direction. Hence, the polycarbonate will not crystallize to bleed out on the surface of the photosensitive layer being formed and deterioration of characteristics such as yield loss due to abnormal projections and defective image due to toner filming, or premature gelation of the coating solution can be prevented.

Further, the polycarbonates of the general formula (I) and the general formula (II) are impermeable to ozone and will hence reduce the chance of deterioration of the carrier transport material. This advantage is particularly notable in the photoreceptor of the present invention since a constituent layer of the carrier transport layer which is more remote from the electroconductive base has a lower concentration of carrier transport material.

The carrier transport layer may be composed of two or three or more constituent layers. If it is made of three or more constituent layers, the content of carrier transport material is the highest in the constituent layer which is the closest to the electroconductive base, with said concentration being decreased toward the outer surface of the carrier transport layer.

Four basic compositions of the photoreceptor of the present invention are shown schematically in Figs. 1 - 4 for illustrative purposes.

The photoreceptor shown in Fig. 1 comprises an electroconductive base 1 overlaid with a carrier generation layer 2 that in turn is overlaid with a carrier transport layer 3 which is composed of constituent layers 3A and 3B. The electroconductive base 1 of the photoreceptor shown in Fig. 2 is formed of a flexible substrate 1A overlaid with an electroconductive layer 1B. In the photoreceptor shown in Fig. 3, the carrier generation layer 2 is overlaid with the carrier transport layer 3 composed of three constituent layers 3A, 3B and 3C. The photoreceptor shown in Fig. 4 is the same as that shown in Fig. 1 except that an intermediate layer or subbing layer 6 is provided between the carrier generation layer 2 and the electroconductive base 1.

The weight ratio of the content of the carrier transport material to binder material in a constituent layer of said carrier transport layer which is the remotest from the electroconductive base (hereinafter referred to as a outermost constituent layer of the carrier transport layer) (layer 3B in the examples shown in Figs. 1, 2 and 4, and layer 3C in the example shown in Fig. 3) is preferably not higher than 70 wt%, more preferably in the range of 5 - 70 wt%. If the weight ratio of the content of carrier transport material to binder material is adjusted to lie within this range, the strength of the carrier transport layer can be increased without sacrificing its ability to transport carriers.

The weight ratio of the content of carrier transport material to binder material in a constituent layer which is the closest to the electroconductive base (layer 3A in the examples shown in Figs. 1 - 4) is preferably at least 30 wt%, more preferably in the range of 30 - 300 wt%. If the weight ratio of the content of carrier transport material to binder material is adjusted to lie within this range, an increased amount of photocarriers can be injected into the carrier transport layer from the carrier generation layer. It is particularly noteworthy that the content of carrier transport material in this constituent layer can be increased to as high as 300 wt% and this has become possible for two reasons: first, the carrier transport layer is composed of two or more constituent layers, and second, the constituent layer the remotest from the electroconductive base has an increased strength.

The weight ratio of the content of carrier transport. material to binder material in a constituent layer which is the remotest from the electroconductive base preferably differs by at least 1.0 wt% from the weight ratio of the content of carrier transport material to binder material in a constituent layer which is the closest to the electroconductive base.

The binder in each of the constituent layers of the carrier transport layer may be made of a polycarbonate represented by the general formula (I) and/or the general formula (II). This is effective in achieving further increase in the strength of the carrier transport layer.

The materials of which the photoreceptor of the present invention are composed and their recipes are described below. First to be discussed is the polycarbonate having a structural unit represented by the general formula (I) and/or the general formula (II) as the principal recurring unit. Prevention of crystallization of the polycarbonate and the attendant advantages already described can be accomplished on account of the "bulkiness" of R¹ and R² in formula (I) or by the action of the ring formed of Z in formula (II). In connection with this, it is more preferred that R¹ and R² in formula (I) are different from each other.

It is essential with the polycarbonate of formula (I) that at least one of R¹ and R² be a bulky group, preferably having at least 3 carbon atoms, in order to provide steric hindrance in such a way as to prevent orientation of the molecular chain.

Illustrative examples of such "bulky" group are listed below:
(1) where R¹¹ is a hydrogen atom, an alkyl group such as methyl, or an alkyl ester group represented by (̵CH₂)ₘ COOR (where R is an alkyl group, and m ≧ 1);
(2)
(3) an alkyl group represented by -CₘH₂ₘ₊₁ (m ≧ 4); and
(4) an alkyl ester group represented by (̵CH₂)ₘ COOR¹² (where R¹² is an alkyl group, and m ≧ 2).

When either one of R¹ and R² is a bulky group, the other may be a hydrogen atom or an alkyl group such as methyl.

In the general formulas (I) and (II), R³ - R¹⁰ may represent not only a hydrogen atom but also a halogen atom such as Cl, Br or F, an alkyl group such as methyl, and a carbocyclic group such as cyclohexyl.

With the polycarbonate represented by the general formula (II), Z may be an atomic group that forms a 5- or 6-membered carbon ring or heterocyclic ring, such as a cyclohexyl group or a cyclopentyl group. These groups may be partly substituted by acetyl, acetylamino or other groups.

Illustrative examples of the structural units represented by general formulas (I) and (II) are listed below:
The polycarbonates that can be used in the present invention have as the principal recurring unit the structural unit represented by the general formula (I) and/or the structural unit represented by the general formula (II). The principal recurring unit may be a single structural unit represented by general formula (I) or general formula (II) (for example, the structural unit (I-2) may be the sole recurring unit), or two or more structural units represented by general formula (I) and/or general formula (II) may be co-condensed. If necessary, a recurring unit represented by general formula (I) and/or general formula (II) may be co-condensed with minor amounts of different other recurring units with a view to providing improved physical, chemical and electrical characteristics. The resulting polycarbonates of co-condensation type are included within the scope of the present invention as long as they are not detrimental to the purposes of the present invention. Specific examples of such polycarbonates of co-condensation type include a polycarbonate prepared by co-condensing 4,4′-dihydroxyphenyl-1,1-cyclohexane with a minor proportion of bisphenol A, and the product of polycondensation of 4,4′-dihydroxyphenyl-1,1-cyclohexane and an aromatic dicarboxylic acid such as terephthalic acid or isophthalic acid.

Additional examples of polycarbonates that can be used in the present invention are represented by the following general formulas (Ia) and (IIa):
where R¹, R², R³, R⁴, R⁵, R⁶, R⁷, R⁸, R⁹ and R¹⁰ each is same as defined for formulas (I) and (II); n is 10 - 5000, preferably 50 - 2000;
and where R³, R⁴, R⁵, R⁶, R⁷, R⁸, R⁹, R¹⁰, Z and n each is same as defined for general formulas (I) and (II).

The polycarbonate having the structural unit represented by general formula (II) as the principal recurring unit is preferred since it is capable of attaining the objects of the present invention in a more effective way. Particularly advantageous structural units are those identified above by (II-2), (II-4) and (II-9) which have a cyclohexane ring bound to the central carbon atom of the bisphenol A portion, and the structural unit identified by (II-2) is most preferred.

The carrier transport material to be incorporated in the carrier transport layer is described below.

Illustrative carrier transport materials include carbazole derivatives represented by the following general formula (III) and hydrazone compounds represented by the following general formulas (IV) - (VI):
(where R¹³ is a substituted or unsubstituted aryl group; R¹⁴ is a hydrogen atom, a halogen atom, a substituted or unsubstituted alkyl group, an alkoxy group, an amino group, a hydroxyl group or a substituted amino group; and R¹⁵ is a substituted or unsubstituted aryl group, or a substituted or unsubstituted heterocyclic group);
(where R¹⁶ and R¹⁷ each is a hydrogen atom or a halogen atom; R¹⁸ and R¹⁹ each is a substituted or unsubstituted aryl group; and Ar¹ is a substituted or unsubstituted arylene group);
(where R²⁰ is a substituted or unsubstituted aryl group, or a substituted or unsubstituted heterocyclic group; R²¹ is a hydrogen atom, a substituted or unsubstituted alkyl group, or a substituted or unsubstituted aryl group; Q is a hydrogen atom, a halogen atom, an alkyl group, a substituted amino group, an alkoxy group or a cyano group; and p is an integer of 0 or 1);
(where R²² is a substituted or unsubstituted aryl group, or a substituted or unsubstituted heterocyclic group; R²³ is a hydrogen atom, a substituted or unsubstituted alkyl group, or a substituted or unsubstituted aryl group; X′₂ is a hydrogen atom, a halogen atom, an alkyl group, a substituted amino group, an alkoxy group or a cyano group; and q is an integer of 0 or 1).

Carrier transport materials represented by the following general formulas (VII) - (IX) can also be used in the present invention:
(where ℓ is an integer of 0 or 1; R²⁴, R²⁵ and R²⁶ each is a substituted or unsubstituted aryl group; R²⁷ and R²⁸ each is a hydrogen atom, an alkyl group having 1 - 4 carbon atoms, a substituted or unsubstituted aryl or aralkyl group, provided that R²⁷ and R²⁸ are not a hydrogen atom at the same time, and when ℓ is 0, R²⁷ is not a hydrogen atom);
(where R²⁹ and R³⁰ is a substituted or unsubstituted alkyl or phenyl group, with the substituent being an alkyl, alkoxy or phenyl group; R³¹ is a substituted or unsubstituted phenyl, naphthyl, anthryl, fluorenyl or heterocyclic group, with the substituent being an alkyl group, an alkoxy group, a halogen atom, a hydroxyl group or a phenyl group; R³¹' is a hydrogen atom, a substituted or unsubstituted alkyl or phenyl group; and R³², R³³, R³⁴ and R³⁵ each is a hydrogen atom, a halogen atom, an alkyl group, an alkoxy group or an alkylamino group);
(where Ar² and Ar³ each is a substituted or unsubstituted phenyl group, with the substituent being a halogen atom, an alkyl group, a nitro group or an alkoxy group; and Ar⁴ is a substituted or unsubstituted phenyl, naphthyl, anthryl, fluorenyl or heterocyclic group, with the substituent being an alkyl group, an alkoxy group, a halogen atom, a hydroxyl group, an aryloxy group, an aryl group, an amino group, a nitro group, a piperidino group, a morpholino group, a naphthyl group, an anthryl group or a substituted amino group, provided that the last-mentioned substituted amino group has an acyl, alkyl, aryl or aralkyl group as the substituent).

Hydrazone compounds represented by the following general formula (X) may also be used in the present invention:
(where D is a substituted or unsubstituted phenyl group, or a substituted or unsubstituted carbazolyl group, as specifically illustrated by
R³⁶ and R³⁷ each represents a substituted or unsubstituted alkyl group, a substituted or unsubstituted aralkyl group, or a substituted or unsubstituted aryl group (illustrative alkyl groups include methyl, ethyl, propyl and butyl; illustrative aralkyl groups include benzyl and phenethyl; illustrative aryl groups include phenyl, α-naphthyl and β-naphthyl; illustrative substituents include a halogen atom, an alkyl group, an alkoxy group and a substituted amino group such as dimethylamino, diethylamino, dipropylamino or dibenzylamino); R³⁸, R³⁹ and R⁴⁵ each represents the same as R³⁶ and R³⁷; and R⁴⁰, R⁴¹, R⁴², R⁴³, R⁴⁴ and R⁴⁶ each represents an alkyl group, an alkoxy group, a halogen atom, etc.)

The carrier transport materials described above may be synthesized by known methods, one of which comprises performing dehydrative condensation between α, β-unsaturated ketone and phenylhydrazine in the presence of an acid catalyst.

The carrier generation layer (CGL) in the photoreceptor of the present invention contains a carrier generation material (CGM) and polycyclic quinone pigments represented by the following general formulas (XI), (XII) and (XIII) may be used as CGM:
In each of these formulas, X is a halogen atom, a nitro group, a cyano group, an acyl group or a carboxyl group; n is an integer of 0 to 4; and m is an integer of 0 to 6.

These polycyclic quinone pigments can be synthesized by known methods.

Other examples of useful CGM include bisazo compounds represented by the following general formula (XIV):
where Ar⁵ and Ar⁶ each is a substituted or unsubstituted carbocyclic aromatic group, or a substituted or unsubstituted heterocyclic aromatic group; R⁴⁷ and R⁴⁸ each is an electron withdrawing group or a hydrogen atom (at least one of R⁴⁷ and R⁴⁸ is -CN, a halogen such as -Cl or an electron withdrawing group such as -NO₂); and A is
(X is a hydroxyl group,
or -NHSO₂-R⁵² (where R⁵⁰, and R⁵¹ each is a hydrogen atom or a substituted or unsubstituted alkyl group; R⁵² is a substituted or unsubstituted alkyl group, or a substituted or unsubstituted aryl group); Y is a hydrogen atom, a halogen atom, a substituted or unsubstituted alkyl group, an alkoxy group, a carboxyl group, a sulfo group, a substituted or unsubstituted carbamoyl group, or a substituted or unsubstituted sulfamoyl group (provided that Y may assume different groups when m is 2 or more); Z is the atomic group necessary to form a substituted or unsubstituted carbocyclic aromatic ring or a substituted or unsubstituted heterocyclic aromatic ring; R⁴⁹ is a hydrogen atom, a substituted or unsubstituted amino group, a substituted or unsubstituted carbamoyl group, a carboxyl group or an ester thereof; A' is a substituted or unsubstituted aryl group; n is an integer of 1 or 2; and m is an integer of 0 - 4).

Among the bisazo compounds represented by formula (XIV), those which are represented by the following general formula (XIVa) are preferred:
where Ar⁵, Ar⁶ and A have the same meanings as defined for formula (XIV).

More preferred are those compounds wherein Ar⁵ and Ar⁶ in formula (XIVa) each represents a substituted or unsubstituted phenyl group, with the substituent being selected from among an alkyl group such as methyl or ethyl, an alkoxy group such as methoxy or ethoxy, a halogen atom such as chlorine or bromine, a hydroxyl group and a cyano group.

Bisazo compounds represented by the following general formula (XV) are also useful as CGM:
where A is
(where Z is the atomic group necessary to form a substituted or unsubstituted aromatic carbon ring or a substituted or unsubstituted aromatic heterocyclic ring; Y is a hydrogen atom, a hydroxyl group, a carboxyl group, an ester group thereof, a sulfo group, a substituted or unsubstituted carbamoyl group, or a substituted or unsubstituted sulfamoyl group; R⁵³ is a hydrogen atom, a substituted or unsubstituted alkyl group, a substituted or unsubstituted amino group, a substituted or unsubstituted carbamoyl group, a carboxyl group, an ester group thereof, a cyano group; Ar⁷ is a substituted or unsubstituted aryl group; and R⁵⁴ is a substituted or unsubstituted alkyl group, a substituted or unsubstituted aralkyl group, or a substituted or unsubstituted aryl group).

Among the bisazo compounds of formula (XV), fluorenylidene group containing bisazo compounds represented by the following general formula (XVa) are particularly effective:
where R⁵⁵ and R⁵⁶ each is an alkyl group, an alkoxy group or an aryl group; R⁵⁷, R⁵⁸, R⁵⁹, R⁶⁰, R⁶¹ and R⁶² each is a hydrogen atom, a halogen atom, an alkyl group, an alkoxy group, an amino group, a hydroxyl group or an aryl group; and A'' is a substituted or unsubstituted aryl group.

The bisazo compounds of formula (XVa) whose intramolecular carbazole group would contribute sensitizing action are capable of providing high sensitivity, particularly in the longer wavelength range. The combination with the intramolecular carbamoyl group moiety provides an effective coupler which exhibits satisfactory sensitivity characteristics over a broad range of wavelengths, thereby contributing to the fabrication of an efficient photoreceptor for use with a semiconductor laser.

Bisazo compounds represented by the following general formula (XVI) can also be used as carrier generation materials:
where X¹ and X² each is a halogen atom, a substituted or unsubstituted alkyl group, a substituted or unsubstituted alkoxy group, a nitro group, a cyano group, a hydroxyl group or a substituted or unsubstituted amino group, provided that at least one of X¹ and X² is a halogen atom; p and q each represents an integer of 0, 1 or 2, provided that p and q are not zero at the same time and that when p is 2, X¹ may assume the same or different groups, and that when q is 2, X² may assume the same or different groups; and A is a group represented by the following general formula (XVII):
(where Ar⁸ is an aromatic carbocyclic or heterocyclic group having at least one fluorinated hydrocarbon group; Z is the nonmetallic atomic group necessary to form a substituted or unsubstituted aromatic carbon ring or a substituted or unsubstituted aromatic hetero ring); and m and n each represents an integer of 0, 1 or 2, provided that m and n are not zero at the same time.

Examples of the halogen atom represented by X¹ and X² in formula (XVI) include chlorine, bromine, fluorine and iodine atoms. At least one of X¹ and X² has a halogen atom. The alkyl group represented by X¹ and X² is preferably a substituted or unsubstituted alkyl group having 1 - 4 carbon atoms and illustrative examples include methyl, ethyl, β-cyanoethyl, iso-propyl, trifluoromethyl and t-butyl. The alkoxy group represented by X¹ and X² is preferably a substituted or unsubstituted alkoxy group having 1 - 4 carbon atoms and illustrative examples include methoxy, ethoxy, β-chloroethyl and sec-butoxy. The substituted or unsubstituted amino group represented by X¹ and X² include those which are substituted by an alkyl group, an aryl group (preferably phenyl), etc. such as N-methylamino, N-ethylamino, N,N-dimethylamino, N,N-diethylamino, N-phenylamino and N,N-diphenylamino, and those which are substituted by an acyl group, such as acetylamino and p-chlorobenzoylamino.

In formula (XVI), p and q each represents 0, 1 or 2, provided that p and q are not zero at the same time, and the preferred case is where p = 1 and 1 = 0 or where p = 1 and q = 1. When p or q is 2, X¹ and X² may be the same or different.

In formula (XVI), A is represented by the following general formula (XVII):
where Ar⁸ is an aromatic carbocyclic or heterocyclic group having at least one fluorinated hydrocarbon group. The fluorinated hydrocarbon group preferably contains 1 - 4 carbon atoms and may be exemplified by trifluoromethyl, pentafluoroethyl, tetrafluoroethyl, heptafluoropropyl, etc. Trifluoromethyl is more preferred. Illustrative aromatic carbocyclic groups include phenyl, naphthyl and anthryl, with phenyl being preferred. Illustrative aromatic heterocyclic groups include carbazolyl and dibenzofuryl. These aromatic carbocyclic and heterocyclic groups may contain substituents other than the fluorinated hydrocarbon group, and such optional substituents include: a substituted or unsubstituted alkyl group having 1 - 4 carbon atoms such as methyl, ethyl, isopropyl, t-butyl or trifluoromethyl; a substituted or unsubstituted aralkyl group such as benzyl or phenethyl; a halogen atom such as chlorine, bromine, fluorine or iodine; a substituted or unsubstituted alkoxy group having 1 - 4 carbon atoms such as methoxy, ethoxy, isopropoxy, t-butoxy or 2-chloroethoxy; a hydroxyl group; a substituted or unsubstituted aryloxy group such as p-chlorophenoxy or 1-naphtoxy; an acyloxy group such as acetyloxy or p-cyanobenzoyloxy; a carboxyl group or an ester group thereof such as ethoxycarbonyl or m-bromophenoxycarbonyl; a carbamoyl group such as an aminocarbonyl, t-butylaminocarbonyl or anilinocarbonyl; an acyl group such as acetyl or o-nitrobenzoyl; a sulfo group or a sulfamoyl group such as aminosulfonyl, t-butylaminousulfonyl or p-tolylaminosulfonyl; an amino group or an acylamino group such as acetylamino or benzoylamino; a sulfonamido group such as methanesulfonamido or p-toluenesulfonamido; a cyano group; and a nitro group. Among these substituents, the following are preferred: a substituted or unsubstituted alkyl group having 1 - 4 carbon atoms such as methyl, ethyl, isopropyl, t-butyl or trifluoromethyl; a halogen atom such as chlorine, bromine, fluorine or iodine; a substituted or unsubstituted alkoxy group having 1 - 4 carbon atoms such as methoxy, ethoxy, t-butoxy or 2-chloroethoxy; a nitro group; and a cyano group.

In formula (XVII), Z represents the atomic group necessary to form a substituted or unsubstituted aromatic carbon or heterocyclic ring and may specifically be exemplified by the atomic groups necessary to form a substituted or unsubstituted benzene ring, a substituted or unsubstituted naphthalene ring, a substituted or unsubstituted indole ring, a substituted or unsubstituted carbazole ring, etc. The atomic groups necessary to form these rings may have substituents such as those listed in connection with Ar⁸ and preferred examples include a halogen atom ie., chlorine, bromine, fluorine or iodine), a sulfo group and a sulfamoyl group (e.g., aminosulfonyl, p-tolylaminosulfonyl, etc.).

Among the bisazo compounds represented by formula (XVI), those which are represented by the following general formulas (XVIII), (XIX), (XX) and (XXI) are preferred:
where X^{1a}, X^{1b}, X^{2a} and X^{2b} each represents a hydrogen atom, a halogen atom, a substituted or unsubstituted alkyl group, a substituted or unsubstituted alkoxy group, a nitro group, a cyano group, a hydroxyl group or a substituted or unsubstituted amino group, provided that at least one of X^{1a}, X^{1b}, X^{2a} and X^{2b} is a halogen atom, and that X^{1a} and X^{1b} or X^{2a} and X^{2b} may be the same or different; Ar′ has the same meaning as Ar⁸ in formula (XVI); Y has the same meaning as the substituent on Z in formula (XVI).

The bisazo compounds represented by the general formula (XVI) can be easily synthesized by known methods.

### Synthesis Example (synthesis of compound XVI-71 to be shown hereinafter)

2,7-Diamino-4-bromo-9-fluorenone (2.89 g, 0.01 mol.) is dispersed in 10 ml of HCl and 20 ml of water. Under cooling at 5°C or below, a solution having 1.40 g (0.02 mol) of sodium nitrite dissolved in 5 ml of water is added dropwise to the dispersion. Under continued stirring for 1 h at the same temperature, the insoluble matter is removed by filtration and a solution having 4.6 g of ammonium hexafluorophosphate in 50 ml of water is added to the filtrate. The precipitating tetrazonium salt is recovered by filtration and dissolved in 100 ml of N,N-dimethylformamide (DMF). Under cooling at 5°C or below, a solution having 6.62 g (0.02 mol) of 2-hydroxy-3-naphthoic acid-3'-trifluoromethylanilide dissolved in 200 ml of DMF is added dropwise.

Under continued cooling at 5°C or below, a solution having 6 g (0.04 mol) of triethanolamine dissolved in 30 ml of DMF is added dropwise and the mixture is stirred for 1 h at 5°C or below, then for additional 4 h at room temperature. After the reaction, the resulting crystal is recovered by filtration, washed successively with DMF and water and finally dried to obtain the end product in an amount of 8.71 g. This product has the following data of elemental analysis: C = 60.5%, H = 2.77%, and N = 8.63% (calculated values), and C = 60.1%, H = 2.95% and N = 8.72% (found values).

Other compounds can be synthesized by similar procedures; first, corresponding amino compounds are used to make diazonium compounds, which are then reacted with 2-hydroxy-3-naphthoic acid-substituted anilide or 2-hydroxy-3-(substituted phenylcarbamoyl) benzo[a]-substituted or unsubstituted carbazole.

The electroconductive base for use in the present invention may be a sheet of metal selected from among, for example, aluminum, nickel, copper, zinc, palladium, silver, indium, tin, platinum, gold, stainless steel, brass, etc. The electroconductive base can also be made by providing an electroconductive layer on an insulating substrate which is suitably selected from among paper, plastic sheets and other materials that are flexible and that have sufficient strength to withstand bending, tensile and other stresses. The electroconductive layer may be formed by various methods including laminating a metal sheet and vacuum evaporating a metal.

The carrier generation layer may be composed of a carrier generation material (CGM) alone or in combination with a suitable binder resin. If desired, a carrier transport material having high mobility of carriers with a specified or unspecified polarity may be incorporated. Specific methods of forming the carrier generation layer include: vacuum evaporating CGM on the electroconductive base described above and; applying or dip-coating CGM which is dissolved or dispersed in a suitable solvent either alone or together with a suitable binder resin, and drying the coating. In the latter method, a binder resin or a carrier transport material may be incorporated and in this case, the proportions of carrier generation material, binder resin and carrier transport material are preferably in the range of 1:(0 - 100):(0 - 500), more preferably in the range of 1:(1 - 10):(0 - 50), on a weight basis.

Constituent layers of the carrier transport layer may be formed by the following process: dissolving or dispersing a carrier transport material and a binder resin in a solvent; coating the solution or dispersion onto the carrier generation layer or other constituent layers of the carrier transport layer; and drying the coated layers.

An intermediate layer or a subbing layer can be formed by coating and drying a solution having a binder resin dissolved in a solvent. Illustrative solvents or dispersants that may be used in this method include: n-butylamine, diethylamine, ethylenediamine isopropanolamine, monoethanolamine, triethanolamine, triethylenediamine, N,N-dimethylformamide, acetone, methyl ethyl ketone, cyclohexanone, benzene, toluene, xylene, chloroform, 1,2-dichloroethane dichloromethane, tetrahydrofuran, dioxane, methanol, ethanol, isopropanol, ethyl acetate, butyl acetate and dimethyl sulfoxide.

Besides the polycarbonates having a structural unit represented by the general formula (I) and/or the general formula (II) as the principal recurring unit, the following resins may be used as binders either on their own or as admixtures: polycarbonates other than those described above, polyesters, methacrylic resins, acrylic resins, polyvinyl chloride, polyvinylidene chloride, polystyrene, polyvinyl acetate, melamine resins, polyurethanes, styrene-acrylate copolymers, styrene-butadiene copolymer, vinylidene chloride-acrylonitrile copolymer, vinyl chloride-vinyl acetate copolymer, vinyl chloride-vinyl acetate-maleic anhydride copolymer, silicone resins, silicone-alkyd resins, phenolic resins, styrene-alkyd resins, poly-N-vinylcarbazole, and polyvinyl butyral.

Other useful resins are transparent resins having a volume resistivity of at least 10⁸Ω·cm, preferably at least 10¹⁰Ω·cm, more preferably at least 10¹³Ω·cm. Resins that cure by the action of light or heat may also the used as binders and examples of such photo- or heat-curable resins include thermosetting acrylic resins, epoxy resins, urethane resins, urea resins, polyester resins, alkyd resins, melamine resins and photocurable cinnamic ester resins, as well as copolymerized and condensed resins thereof. All other photo- and heat-curable resins commonly employed in electrophotographic materials may be used in the present invention. In order to provide improved working and physical properties (e.g. prevention of cracking and imparting flexibility), the protective layer may incorporate therein less than 50 wt% of a thermoplastic resin as required. Usable thermoplastic resins include, for example, polypropylene, acrylic resins, methacrylic resins, vinyl chloride resin, vinyl acetate resin, epoxy resins, polycarbonate resins, copolymerized resins thereof, high-molecular weight organic semiconductors such as poly-N-vinylcarbazole, and any other thermoplastic resins that are commonly used in electrophotographic materials.

Binder resins that are to be used in an intermediate layer or a subbing layer may be selected from among metal oxides such as aluminum oxide and indium oxide and high-molecular weight materials such as acrylic resins, methacrylic resins, vinyl chloride resin, vinyl acetate resin, epoxy resins, polyurethane resins, phenolic resins, polyester resins, alkyd resins, polycarbonate resins, silicone resins, melamine resins, vinyl chloride-vinyl acetate copolymer resin, and vinyl chloride-vinyl acetate-maleic anhydride copolymer resin.

Speaking of the photoreceptors shown in Figs. 1 - 4, the constituent layers 3A, 3B and 3C of the carrier transport layer 3 may employ the same or different binder resins. For example, in order to provide improved light sensitivity, the topmost or outermost constituent layer 3B or 3C may use the polycarbonate of the present invention, with a bisphenol A type polycarbonate being used in the bottommost constituent layer 3A that is the closest to the electroconductive base. If desired, the constituent layer 3A (or 3B) which is adjacent the outermost constituent layer 3B (or 3C) and which is closer to the electro conductive base may be designed to employ a binder resin that is hardly soluble with respect to the solvent used to coat said outermost constituent layer. This offers the advantage of preventing not only diffusion of the carrier transport material into the bottommost constituent layer 3A but also swelling of said layer.

The constituent layer 3B or 3C that is more remote from the electroconductive base may be coated in a different way than the bottommost constituent layer 3A is coated. For instance, the constituent layer 3A may be formed by dip coating whereas the constituent layer 3B or 3C is formed by spray coating, and this is effective in preventing dissolution and swelling of the bottommost constituent layer 3A.

The bottommost constituent layer 3A preferably has a thickness of 5 - 50 µm, with the range of 5 - 30 µm being more preferred. The outermost constituent layer 3B or 3C preferably has a thickness of 0.1 - 30 µm, with the range of 0.5 - 10 µm being more preferred.

The carrier generation layer preferably has a thickness of 0.01 - 10 µm, with the range of 0.1 - 5 µm being more preferred.

The light-sensitive layer may have a high-molecular weight semiconductor contained therein. While various high-molecular weight semiconductors may be used, poly-N-vinylcarbazole and its derivatives are preferred because of their high degree of curability. Derivatives of poly-N-vinylcarbazole are such that all or part of the carbazole rings in the recurring units have various substituents such as an alkyl group, a nitro group, an amino group, a hydroxyl group and a halogen atom.

The light-sensitive layer may also have at least one electron - accepting materials contained therein in order to attain various purposes such as improving sensitivity, reducing residual potential and minimizing fatigue that results from cyclic use of the photoreceptor. Exemplary electron-accepting materials that may be used in the photoreceptor of the present invention include: succinic anhydride, maleic anhydride, dibromomaleic anhydride, phthalic anhydride, tetrachlorophthalic anhydride, tetrabromophthalic anhydride, 3-nitrophthalic anhydride, 4-nitrophthalic anhydride, pyromellitic anhydride, mellitic anhydride, tetracyanoethylene, tetracyanoquinodimethane, o-dinitrobenzene, m-dinitrobenzene, 1,3,5-trinitrobenzene, paranitrobenzonitrile, picryl chloride, quinone chlorimide, chloranyl, bromanyl, 2-methylnaphthoquinone, dichlorodicyanoparabenzoquinone, anthraquinone, dinitroanthraquinone, trinitrofluorenone, 9-fluorenylidene-(dicyanomethylenemalonodinitrile), polynitro-9-fluorenylidene-(dicyanomethylenemalonodinitrile), picric acid, o-nitrobenzoic acid, p-nitrobenzoic acid, 3,5-dinitrobenzoic acid, pentafluorobenzoic acid, 5-nitrosalicylic acid, 3,5-dinitrosalicylic acid, phthalic acid, mellitic acid and other compounds having a high degree of electron affinity. These electron-accepting substances may be used either on their own or as admixtures. Among these examples, fluorenone compounds, quinone compounds and benzene derivatives having electron-withdrawing substituents such as Cl, CN and NO₂ may be used with particular advantage.

Silicone oil and fluorine containing surfactants may also be incorporated as surface modifiers in the photoreceptor of the present invention. Ammonium compounds may also be incorporated as agents to provide improved durability. Ultraviolet (uv) absorbers may also be incorporated and preferred examples include benzoic acid, stilbene compounds and their derivatives, and nitrogenous compounds such as triazole compounds, imidazole compounds, triazine compounds, coumarin compounds, oxadiazole compounds, thiazole compounds and derivatives thereof.

An antioxidant may be incorporated in the carrier transport layer, the carrier generation layer and the light-sensitive layer. This is effective not only in minimizing the adverse effects of ozone that is generated by discharging but also in preventing the increase in residual potential or decrease in charging potential that might occur during cyclic use of the photoreceptor. Illustrative antioxidants include hindered phenol, hindered amines, paraphenylenediamine, arylalkanes, hydroquinone, spirochromans, spiroindanone and its derivatives, organosulfur compounds, and organo-phosphorus compounds.

The following examples are provided for the purpose of further illustrating the present invention but are in no way to be taken as limiting.

### Preparation of electrophotographic photoreceptors:

Samples of electrophotographic photoreceptor were prepared as described below.

### EXAMPLE 1

A 100-µm thick electroconductive base made of aluminum-evaporated polyethylene terephthalate was coated with an intermediate layer ca. 0.1 µm thick that was made of a vinyl chloride-vinyl acetate-maleic anhydride copolymer. ("ES-lac MF-10" of Sekisui Chemical Co., Ltd.) In the next step, 4 g of a polycyclic quinone pigment having the structural formula XI-3 shown below was pulverized in a ball mill for 24 h. To the resulting particles, a solution having 2 g of a bisphenol A type polycarbonate ("Panlite L-1250" of Teijin Ltd.) dissolved in 130 ml of 1,2-dichloroethane was added. The mixture was stirred for an additional 24 h to form a dispersion, which was coated by doctor blading onto the previously formed intermediate layer and dried to form a carrier generation layer (CGL) in a thickness of Ca. 0.5 µm.

In the next step, 8 g of a styryl compound (carrier transport material) represented by the structural formula VIII-35 shown hereinafter and 10 g of a polycarbonate ("Panlite L-1250") were dissolved in 100 ml of 1,2-dichloroethane. The resulting solution was coated by doctor blading onto the carrier generation layer and dried at 80°C for 1 h to form a constituent layer of carrier transport layer that was the closest to the electroconductive base in thickness of 18 µm. In this constituent layer, the weight ratio of the content of carrier transport material to binder resin was 80 wt%.

In the next step, 6 g of a styryl compound represented by the structural formula VIII-35 and 10 g of a polycarbonate (viscosity average mol. wt. ca. 30,000) composed of recurring units represented by the structural formula II-2 were dissolved in 100 ml of monochlorobenzene. The resulting solution was coated by doctor blading onto the constituent layer of carrier transport layer that was the closest to the electroconductive base to form the outermost constituent layer of carrier transport layer in a thickness of 4 µm. In this outermost constituent layer, the weight ratio of the content of carrier transport material to binder resin was 60 wt%. Since the solubility of the polycarbonate "Panlite L-1250" in monochlorobenzene was smaller than that of the polycarbonate composed of recurring units represented by the structural formula II-2, the constituent layer of carrier transport layer that was the closest to the electroconductive base would not readily dissolve when the outermost constituent layer was being applied.

### EXAMPLE 1A

An electrophotographic photoreceptor was fabricated as in Example 1 except that the amount of the carrier transport material in the constituent layer of carrier transport layer that was the closest to the electroconductive base was changed from 8 g to 20 g (200%).

### EXAMPLE 2

An intermediate layer and a carrier generation layer were formed as in Example 1. The constituent layer of carrier transport layer that was the closest to the electroconductive base was formed as in Example 1 except that the layer thickness was changed to 19 µm.

In the next step, the outermost constituent layer of carrier transport layer was formed as in Example 1 except that the amount of carrier transport material and the layer thickness were changed to 4 g and 3 µm, respectively.

### COMPARATIVE EXAMPLE 1

An intermediate layer and a carrier generation layer were formed as in Example 1.

In the next step, 8 g of a carrier transport material represented by the structural formula VIII-35 and 10 g of a polycarbonate "Panlite L-1250" were dissolved in 100 ml of 1,2-dichloroethane and the resulting solution was coated onto the carrier generation layer to form a single-layered carrier transport layer in a thickness of 22 µm.

### COMPARATIVE EXAMPLE 1A

Another comparative photoreceptor was prepared by the following procedures. In the first step, an intermediate layer and a carrier generation layer were formed as in Example 1. In the next step, the constituent layers of the carrier transport layer that was the closest to the electroconductive base and the outermost constituent layer of the carrier transport layer were successively formed as in Example 1, except that the content of the carrier transport material in the constituent layer of the carrier transport layer that was the closest to the electroconductive base and its thickness were changed to 4 g and 19 µm, respectively, and that the content of the carrier transport material in the outermost constituent layer and its thickness were changed to 8 g and 3 µm, respectively.

### COMPARATIVE EXAMPLE 1B

Still another comparative photoreceptor was prepared as in Example 1 except that a bisphenol A type polycarbonate "Panlite L-1250" was used as a binder resin in the outermost constituent layer of carrier transport layer.

### EXAMPLE 3

An intermediate layer and a carrier generation layer were formed as in Example 1 except that a fluorenone compound represented by the structural formula XVI-71 shown hereinafter was used as a carrier generation material.

In the next place, 10 g of a polycarbonate composed of recurring units represented by the general structural formula II-2 and 10 g of a carrier transport material represented by the structural formula VIII-38 also shown hereinafter were dissolved in 100 ml of monochlorobenzene. The resulting solution was coated onto the carrier generation layer to form a constituent layer of the carrier transport layer that was the closest to the electroconductive base in a thickness of 15 µm.

A coating solution for the outermost constituent layer was prepared as described above except that the content of the carrier transport material was reduced to 7 g. This solution was spray-coated onto the constituent layer of the carrier transport layer that was the closest to the electroconductive base to form the outermost constituent layer in a thickness of 5 µm.

### EXAMPLE 4

An electrophotographic photoreceptor was prepared as in Example 3, except that the thickness of the constituent layer of the carrier transport layer that was the closest to the electroconductive base, the content of the carrier transport material in the outermost constituent layer and its thickness were changed to 17 µm, 5 g and 3 µm, respectively.

### EXAMPLE 5

An electrophotographic photoreceptor was prepared as in Example 3, except that the thickness of the constituent layer of the carrier transport layer that was the closest to the electroconductive base, the content of the carrier transport material in the outermost constituent layer and its thickness were changed to 18 µm, 3 g and 2 µm, respectively.

### COMPARATIVE EXAMPLE 3

An intermediate layer and a carrier generation layer were formed as in Example 3.

In the next step, a coating solution of the same composition as that of the solution for forming the constituent layer of carrier transport layer that was the closest to the electroconductive base in Example 3 (containing 10 g of the carrier transport material) was coated onto the carrier generation layer by doctor blading to form a single-layered carrier transport layer in a thickness of 20 µm.

### COMPARATIVE EXAMPLE 4

An additional comparative electrophotographic photoreceptor was prepared as in Comparative Example 3 except that the content of the carrier transport material in the carrier transport layer was changed to 3 g.

### EXAMPLE 6

An intermediate layer was formed as in Example 1.

In the next step, a carrier generation layer was formed as in Example 1 except that a bisazo compound represented by the structural formula XIV-5 shown hereinafter was used as a carrier generation material and that a polyester resin "Vylon-200" of Toyobo Co., Ltd. was used as a binder resin.

Subsequently, 10 g of a carrier transport material having the structural formula X-2 shown hereinafter and 10 g of poly-N-vinylcarbazole "Ruvican M-170" of BASE A.G. were dissolved in 100 ml of tetrahydrofuran (THF) and the resulting solution was coated onto the carrier generation layer by doctor blading to form the constituent layer of carrier transport layer that was the closest to the electroconductive base in a thickness of 18 µm.

In the next place, 6 g of a carrier transport material represented by the structural formula X-2 and 10 g of a polycarbonate composed of structural units represented by the formula II-2 were dissolved in 100 ml of 1,2-dichloroethane, and the resulting solution was coated onto the constituent layer that was closest to the electroconductive base by doctor blading to form the outermost constituent layer in a thickness of 4 µm.

### EXAMPLE 7

An electrophotographic photoreceptor was prepared as in Example 6, except that the thickness of the constituent layer of carrier transport layer that was the closest to the electroconductive base, the thickness of the outermost constituent layer and the weight ratio of the content of carrier transport material to binder resin in the outermost constituent layer were changed to 19 µm, 3 µm and 40%, respectively.

### COMPARATIVE EXAMPLE 6

An intermediate layer and a carrier generation layer were formed as in Example 6. In the next step, a coating solution of the same composition as that of the solution for forming the constituent layer of carrier transport layer that was the closest to the electroconductive base in Example 6 was prepared and coated onto the carrier generation layer by doctor blading to form a single-layered carrier transport layer in a thickness of 22 µm.

### EXAMPLE 8

An intermediate layer and a carrier generation layer were formed as in Example 1.

In the next step, 8 g of a pyrazoline compound represented by the structural formula VII-22 shown below and 10 g of a polycarbonate "Panlite L-1250" were dissolved in 100 ml of 1,2-dichloroethane and the resulting solution was coated onto the carrier generation layer to form the constituent layer of carrier transport layer that was the closest to the electroconductive base in a thickness of 18 µm.

Subsequently, 6 g of a pyrazoline compound represented by the structural formula VII-22 and 10 g of a polycarbonate composed of structural units represented by the formula II-5 were dissolved in 100 ml of monochlorobenzene, and the resulting solution was coated onto the constituent layer of carrier transport layer that was the closest to the electroconductive base by doctor blading to form the outermost constituent layer in a thickness of 4 µm.

### Structural formulas

### Evaluating the characteristics of photoreceptors:

The samples of electrophotographic photoreceptors prepared in Examples 1 - 8 and Comparative Examples 1 - 6 were set on a copying machine adapted from U-Bix 1550 MR of Konica Corp. and a copying test was conducted through 5 x 10⁴ cycles. At the same time, measurements were conducted for black paper potential V_{B} and white paper potential V_{W}. After taking 5 x 10⁴ copies, checking was made for the amount of decrease in photoreceptor's thickness by wear and for the occurrence of scratches on image surface. The values of V_{B} and V_{W} measured before copying and after copying 5 x 10⁴ sheets, as well as the variations in the respective values (Δ|V_{B}| and Δ|V_{W}|) are shown in Fig. 5.

The term "black paper potential" means the surface potential which developed on a photoreceptor when it was subjected to the cyclic copying test described above using a black paper original having a reflection density of 1.3. The term "white paper potential" means the surface potential which developed on the same photoreceptor when used with a white paper original.

As the data in Fig. 5 shows, the photoreceptor samples prepared in Examples 1 - 8 were high in wear and scratch resistance, showed satisfactory values of both black paper and white paper potential, and permitted a great number of copies to be taken to produce image of consistent quality with minimum variations in the values of black paper and white paper potential.

## Claims

1. A photoreceptor having an electroconductive base, a carrier generation layer formed thereon, and carrier transport layer overlaid on the carrier generation layer and containing a carrier transport material and a binder material; the carrier transport layer comprising at least two constituent layers, so that the weight ratio of the carrier transport material to the binder material in a continuous layer which is closer to the electroconductive base is higher than the weight ratio of the carrier transport material in a constituent layer which is more remote from the electroconductive base, and a polycarbonate having as the principal recurring unit a structural unit represented by formula (I) or a structural unit represented by formula (II) contained in the binder material in the outermost constituent layer of the carrier transport layer: wherein R¹ and R² are each a hydrogen atom, a substituted or unsubstituted aliphatic group, a substituted or unsubstituted aromatic group; R³, R⁴, R⁵, R⁶, R⁷, R⁸, R⁹ and R¹⁰ are each a hydrogen atom, a halogen atom, a substituted or unsubstituted aliphatic group, a substituted or unsubstituted carbocyclic group; wherein Z is the group of atoms necessary to form a substituted or unsubstituted carbon ring or a substituted or unsubstituted heterocyclic ring; and at least one of R¹ or R² is a member selected from groups (1) to (4) below,
(1) wherein R¹¹ is a hydrogen atom, an alkyl group, or an alkyl ester group represented by -(CH₂)ₘCOOR, wherein R is an alkyl group, and m ≧ 1;
(2)
(3) an alkyl group represented by -CₘH₂ₘ₊₁ where m ≧ 4; and
(4) an alkyl ester group represented by -(CH₂)ₘCOOR¹², wherein R¹² is an alkyl group and m ≧ 2.

2. A photoreceptor according to claim 1 characterised in that the ratio of the carrier transport material to the binder material in a constituent layer which is the closest to the electroconductive base is higher than the weight ratio of the ratio of the carrier transport material to the binder material in the outermost constituent layer of the carrier transport layer, with the difference between the two weight ratios being at least 20%.

3. A photoreceptor according to claim 2 characterised in that the weight ratio of the carrier transport material to binder material in a constituent layer which is the closest to the electroconductive base is higher than the weight ratio of the carrier transport material to the binder material in the outermost constituent layer of the carrier transport layer, with the difference between the two weight ratios lying in the range 20% to 140%.

4. A photoreceptor according to claim 1 characterised in that the carrier transport layer contains a polycarbonate having at least the structural unit represented by formula (II) as the principal recurring unit.

5. A photoreceptor according to claim 1 characterised in that the outermost constituent layer of the carrier transport layer has the carrier transport material in an amount of not more than 70% by weight of the binder material in the outermost constituent layer of the carrier transport layer.

6. A photoreceptor according to claim 5 characterised in that the outermost constituent layer of the carrier transport layer has the carrier transport material in an amount of 5% to 70% by weight of the binder material in the outermost constituent layer of the carrier transport layer.

7. A photoreceptor according to claim 1 characterised in that the constituent layer of the carrier transport layer which is the closest to the electroconductive base has the carrier transport material in an amount of more than 30% by weight of the binder material in the constituent layer of the carrier transport layer which is the closest to the electroconductive base.

8. A photoreceptor according to claim 7 characterised in that the constituent layer of the carrier transport layer which is the closest to the electroconductive base has the carrier transport material in an amount of 30% to 300% by weight of the binder material in the constituent layer of the carrier transport layer which is the closest to the electroconductive base.

9. A photoreceptor according to claim 1 characterised in that R¹ and R² in the general formula (I) represent different groups.

10. A photoreceptor according to claim 1 characterised in that at least one of R¹ and R² in the general formula (I) is a bulky group having at least 3 carbon atoms.

11. A photoreceptor according to claim 1 characterised in that each of the groups R³ to R¹⁰ in the general formulas (I) and (II) is a hydrogen atom, a halogen atom, a methyl group or a cyclohexyl group.

12. A photoreceptor according to claim 1 characterised in that Z in the general formula (II) forms a 5- or 6-membered carbon ring or heterocyclic ring.

13. A photoreceptor according to claim 1 characterised in that the number of repetitions of the structural unit represented by the general formulas (I) or (II) is from 10 to 5000.

14. A photoreceptor according to claim 13 characterised in that the number of repetitions of the structural unit represented by the general formulas (I) or (II) is from 50 to 2000.

15. A photoreceptor according to claim 1 characterised in that the polycarbonate has at least a structural unit represented by the general formula (II).

16. A photoreceptor according to claim 12 characterised in that the groups R³ to R¹⁰ in the general formula (II) are each a hydrogen atom and Z represents the group of atoms necessary to form a cyclohexylidene ring.

17. A photoreceptor according to claim 1 characterised in that the carrier transport material is at least one of the compounds represented by the following general formulas (III) to (X): (where R¹³ is a substituted or unsubstituted aryl group; R¹⁴ is a hydrogen atom, a halogen atom, a substituted or unsubstituted alkyl group, an alkoxy group, an amino group, a hydroxyl group or a substituted amino group; and R¹⁵ is a substituted or unsubstituted aryl group, or a substituted or unsubstituted heterocyclic group); (where R¹⁶ and R¹⁷ each is a hydrogen atom or a halogen atom; R¹⁸ and R¹⁹ each is a substituted or unsubstituted aryl group; and Ar¹ is a substituted or unsubstituted arylene group); (where R²⁰ is a substituted or unsubstituted aryl group, or a substituted or unsubstituted heterocyclic group; R²¹ is a hydrogen atom, a substituted or unsubstituted alkyl group, or a substituted or unsubstituted aryl group; Q is a hydrogen atom, a halogen atom, an alkyl group, a substituted amino group, an alkoxy group or a cyano group; and p is an integer of 0 or 1); (where R²² is a substituted or unsubstituted aryl group, or a substituted or unsubstituted heterocyclic group; R²³ is a hydrogen atom, a substituted or unsubstituted alkyl group, or a substituted or unsubstituted aryl group; X'₂ is a hydrogen atom, a halogen atom, an alkyl group, a substituted amino group, an alkoxy group or a cyano group; and q is an integer of 0 or 1); (where ℓ is an integer of 0 or 1; R²⁴, R²⁵ and R²⁶ each is a substituted or unsubstituted aryl group; R²⁷ and R²⁸ each is a hydrogen atom, an alkyl group having 1 - 4 carbon atoms, a substituted or unsubstituted aryl or aralkyl group, provided that R²⁷ and R²⁸ are not a hydrogen atom at the same time, and when ℓ is 0, R²⁷ is not a hydrogen atom); (where R²⁹ and R³⁰ each is a substituted or unsubstituted alkyl or phenyl group, with the substituent being an alkyl, alkoxy or phenyl group; R³¹ is a substituted or unsubstituted phenyl, naphthyl, anthryl, fluorenyl or heterocyclic group, with the substituent being an alkyl group, an alkoxy group, a halogen atom, a hydroxyl group or a phenyl group; R³¹' is a hydrogen atom, a substituted or unsubstituted alkyl or phenyl group; and R³², R³³, R³⁴ and R³⁵ each is a hydrogen atom, a halogen atom, an alkyl group, an alkoxy group or an alkylamino group); (where Ar² and Ar³ each is a substituted or unsubstituted phenyl group, with the substituent being a halogen atom, an alkyl group, a nitro group or an alkoxy group; and Ar⁴ is a substituted or unsubstituted phenyl, naphthyl, anthryl, fluorenyl or heterocyclic group, with the substituent being an alkyl group, an alkoxy group, a halogen atom, a hydroxyl group, an aryloxy group, an aryl group, an amino group, a nitro group, a piperidino group, a morpholino group, a naphthyl group, an anthryl group or a substituted amino group, in which the substituent is an acyl, an alkyl, an aryl, or an aralkyl group; where D is a substituted or unsubstituted phenyl group or a substituted or unsubstituted carbazolyl group, or a group selected from the groups: where R³⁶, R³⁷, R³⁸, R³⁹ and R⁴⁵ each represents a substituted or unsubstituted alkyl group, a substituted or unsubstituted aralkyl group or a substituted or unsubstituted aryl group; and R⁴⁰, R⁴¹, R⁴², R⁴³, R⁴⁴ and R⁴⁶ each represents an alkyl group, an alkoxy group, or a halogen atom .

18. A photoreceptor according to claim 1 wherein the carrier generation material contained in said carrier generation layer is a polycyclic quinone pigment or a bisazo pigment.

19. A photoreceptor according to claim 16 wherein said polycyclic quinone pigment is anthanthrone pigment represented by the following general formula (XI): where X is a halogen atom, a nitro group, a cyano group, an acyl group or a carboxyl group; n is an integer of 0 to 4; and m is an integer of 0 to 6.

20. A photoreceptor according to claim 16 wherein said bisazo pigment is fluorenylidene pigment represented by the following general formula (XVa): where R⁵⁵ and R⁵⁶ each is an alkyl group, an alkoxy group or an aryl group; R⁵⁷, R⁵⁸, R⁵⁹, R⁶⁰, R⁶¹ and R⁶² each is a hydrogen atom, a halogen atom, an alkyl group, an alkoxy group, an amino group, a hydroxyl group or an aryl group; and A'' is a substituted or unsubstituted aryl group.

21. A photoreceptor according to claim 16 wherein said bisazo pigment is a fluorenone pigment represented by the following general formula (XVI): where X¹ and X² each is a halogen atom, a substituted or unsubstituted alkyl group, a substituted or unsubstituted alkoxy group, a nitro group, a cyano group, a hydroxyl group or a substituted or unsubstituted amino group, provided that at least one of X¹ and X² is a halogen atom; p and q each represents an integer of 0, 1 or 2, provided that p and q are not zero at the same time and that when p is 2, X¹ may be the same or different groups, and that when q is 2, X² may be the same or different groups; and A is a group represented by the following general formula (XVII): (where Ar⁸ is an aromatic carbocyclic or heterocyclic group having at least one fluorinated hydrocarbon group; Z represents the nonmetallic atoms necessary to form a substituted or unsubstituted aromatic carbon ring or a substituted or unsubstituted aromatic heterocyclic ring); m and n each represents an integer of 0, 1 or 2, provided that m and n are not zero at the same time.

22. A photoreceptor according to claim 1 wherein a constituent layer of said carrier transport layer that is closer to the electroconductive base and that is adjacent to the outermost constituent layer of said carrier transport layer contains a bisphenol A type polycarbonate as a binder.

23. A photoreceptor according to claim 1 wherein the binder resin contained in a constituent layer of said carrier transport layer that is closer to the electroconductive base and that is adjacent to the outermost constituent layer of said carrier transport layer is hardly soluble with respect to the solvent used to coat said outermost constituent layer.

24. A photoreceptor according to claim 1 wherein a constituent layer of said carrier transport layer that is the closest to the electroconductive base is formed by dip coating, and a constituent layer of said carrier transport layer that is adjacent to said constituent layer and that is more remote from the electroconductive base is formed by spray coating.

25. A photoreceptor according to claim 1 wherein a constituent layer of said carrier transport layer which is the closest to the conductive base has a thickness of 5 - 50 µm.

26. A photoreceptor according to claim 1 wherein a constituent layer of said carrier transport layer which is the closest to the electroconductive base has a thickness of 5 - 30 µm.

27. A photoreceptor according to claim 1 wherein the outermost constituent layer of said carrier transport layer has a thickness of 0.1 - 30 µm.

28. A photoreceptor according to claim 1 wherein the outermost constituent layer of said carrier transport layer has a thickness of 0.5 - 10 µm.

29. A photoreceptor according to claim 1 wherein said carrier generation layer has a thickness of 0.01 - 10 µm.

30. A photoreceptor according to claim 1 wherein said carrier generation layer has a thickness of 0.1 - 5 µm.

## Patentansprüche

1. Photorezeptor mit einem elektrisch leitfähigen Träger, einer darauf gebildeten Ladungsträgererzeugungsschicht und einer die Ladungsträgererzeugungsschicht überlagernden und ein Ladungsträgertransportmaterial und ein Bindemittel enthaltenden Ladungsträgertransportschicht, wobei die Ladungsträgertransportschicht mindestens zwei dieselbe aufbauende Schichten umfaßt, so daß das Gewichtsverhältnis des Ladungsträgertransportmaterials zum Bindemittel in einer durchgehenden Schicht, die näher an der elektrisch leitfähigen Basis liegt, höher ist als das Gewichtsverhältnis des Ladungsträgertransportmaterials in einer aufbauenden Schicht, die von dem elektrisch leitfähigen Träger weiter entfernt liegt, und einem Polycarbonat, das als die Hauptrepetiereinheit eine durch die Formel (I) dargestellte Struktureinheit oder eine durch die Formel (II) dargestellte Struktureinheit im Bindemittel in der äußersten aufbauenden Schicht der Ladungsträgertransportschicht: aufweist, wobei R¹ und R² jeweils ein Wasserstoffatom, eine gegebenenfalls substituierte aliphatische Gruppe, eine gegebenenfalls substituierte aromatische Gruppe darstellen; R³, R⁴, R⁵, R⁶, R⁷, R⁸, R⁹ und R¹⁰ jeweils ein Wasserstoffatom, ein Halogenatom, eine gegebenenfalls substituierte aliphatische Gruppe, eine gegebenenfalls substituierte carbocyclische Gruppe darstellen; wobei Z die zur Bildung eines gegebenenfalls substituierten Kohlenstoffrings oder eines gegebenenfalls substituierten heterocyclischen Rings nötige Gruppe von Atomen darstellt; und wenigstens eines von R¹ und R² den unten angeführten Gruppen (1) bis (4) angehört,
(1) wobei R¹¹ ein Wasserstoffatom, eine Alkylgruppe oder eine durch -(CH₂)ₙCOOR dargestellte Alkylestergruppe ist, wobei R eine Alkylgruppe ist, und m ≧ 1;
(2)
(3) eine durch -CₘH₂ₘ₊₁ dargestellte Alkylgruppe ist, wobei m ≧ 4; und
(4) eine durch -(CH₂)ₘCOOR¹² dargestellte Alkylestergruppe ist, wobei R¹² eine Alkylgruppe ist und m ≧ 2.

2. Photorezeptor gemäß Anspruch 1, dadurch gekennzeichnet, daß das Verhältnis des Ladungsträgertransportmaterials zum Bindemittel in einer dem elektrisch leitfähigen Träger am nächsten liegenden aufbauenden Schicht höher ist als das Gewichtsverhältnis des Ladungsträgertransportmaterials zum Bindemittel in der äußersten aufbauenden Schicht der Ladungsträgertransportschicht, wobei der Unterschied zwischen den zwei Gewichtsverhältnissen wenigstens 20% beträgt.

3. Photorezeptor gemäß Anspruch 2, dadurch gekennzeichnet, daß das Gewichtsverhältnis des Ladungsträgertransportmaterials zum Bindemittel in einer dem elektrisch leitfähigen Träger am nächsten liegenden aufbauenden Schicht höher ist als das Gewichtsverhältnis des Ladungsträgertransportmaterials zum Bindemittel in der äußersten aufbauenden Schicht der Ladungsträgertransportschicht, wobei der Unterschied zwischen den zwei Gewichtsverhältnissen im Bereich zwischen 20 % und 140% liegt.

4. Photorezeptor gemäß Anspruch 1, dadurch gekennzeichnet, daß die Ladungsträgertransportschicht ein wenigstens die durch Formel (II) dargestellte Struktureinheit als die Hauptrepetiereinheit aufweisendes Polycarbonat enthält.

5. Photorezeptor gemäß Anspruch 1, dadurch gekennzeichnet, daß die äußerste aufbauende Schicht der Ladungsträgertransportschicht das Ladungsträgertransportmaterial in einer Menge von nicht über 70 Gew.-% des Bindemittels in der äußersten aufbauenden Schicht der Ladungsträgertransportschicht aufweist.

6. Photorezeptor gemäß Anspruch 5, dadurch gekennzeichnet, daß die äußerste aufbauende Schicht der Ladungsträgertransportschicht das Ladungsträgertransportmaterial in einer Menge von zwischen 5 Gew.-% bis 70 Gew.-% des Bindemittels in der äußersten aufbauenden Schicht der Ladungsträgertransportschicht aufweist.

7. Photorezeptor gemäß Anspruch 1, dadurch gekennzeichnet, daß die dem elektrisch leitfähigen Träger am nächsten gelegene aufbauende Schicht der Ladungsträgertransportschicht das Ladungsträgertransportmaterial in einer Menge von über 30 Gew.-% des Bindemittels in der dem elektrisch leitfähigen Träger am nächsten gelegenen aufbauenden Schicht der Ladungsträgertransportschicht aufweist.

8. Photorezeptor gemäß Anspruch 7, dadurch gekennzeichnet, daß die dem elektrisch leitfähigen Träger am nächsten gelegene aufbauende Schicht der Ladungsträgertransportschicht das Ladungsträgertransportmaterial in einer Menge von zwischen 30 Gew.-% und 300 Gew.-% des Bindemittels in der dem elektrisch leitfähigen Träger am nächsten gelegenen aufbauenden Schicht der Ladungsträgertransportschicht aufweist.

9. Photorezeptor gemäß Anspruch 1, dadurch gekennzeichnet, daß R¹ und R² in der allgemeinen Formel (I) verschiedene Gruppen darstellen.

10. Photorezeptor gemäß Anspruch 1, dadurch gekennzeichnet, daß wenigstens eines von R¹ und R² in der allgemeinen Formel (I) eine sperrige Gruppe mit wenigstens 3 Kohlenstoffatomen bedeutet.

11. Photorezeptor gemäß Anspruch 1, dadurch gekennzeichnet, daß die Gruppen R³ bis R¹⁰ in den allgemeinen Formeln (I) und (II) jeweils ein Wasserstoffatom, ein Halogenatom, eine Methylgruppe oder eine Cyclohexylgruppe bedeutet.

12. Photorezeptor gemäß Anspruch 1, dadurch gekennzeichnet, daß Z in der allgemeinen Formel (II) einen 5- oder 6-gliedrigen Kohlenstoffring oder heterocyclischen Ring bildet.

13. Photorezeptor gemäß Anspruch 1, dadurch gekennzeichnet, daß die Anzahl von Wiederholungen der durch die allgemeine Formel (I) oder (II) dargestellten Struktureinheit zwischen 10 und 5000 liegt.

14. Photorezeptor gemäß Anspruch 13, dadurch gekennzeichnet, daß die Anzahl von Wiederholungen der durch die allgemeine Formel (I) oder (II) dargestellten Struktureinheit zwischen 50 und 2000 liegt.

15. Photorezeptor gemäß Anspruch 1, dadurch gekennzeichnet, daß das Polycarbonat wenigstens eine durch die allgemeine Formel (II) dargestellte struktureinheit aufweist.

16. Photorezeptor gemäß Anspruch 12, dadurch gekennzeichnet, daß die Gruppen R³ bis R¹⁰ in der allgemeinen Formel (II) jeweils ein Wasserstoffatom bedeuten und Z die zur Bildung eines Cyclohexylidenrings nötige Gruppe von Atomen darstellt.

17. Photorezeptor gemäß Anspruch 1, dadurch gekennzeichnet, daß es sich bei dem Ladungsträgertransportmaterial um wenigstens eine der durch die nachfolgenden allgemeinen Formeln (III) bis (X) dargestellten Verbindungen handelt: (wobei R¹³ eine gegebenenfalls substituierte Arylgruppe bedeutet; R¹⁴ ein Wasserstoffatom, ein Halogenatom, eine gegebenenfalls substituierte Alkylgruppe, eine Alkoxygruppe, eine Aminogruppe, eine Hydroxylgruppe oder eine substituierte Aminogruppe bedeutet; und R¹⁵ eine gegebenenfalls substituierte Arylgruppe oder eine gegebenenfalls substituierte heterocyclische Gruppe bedeutet); (wobei R¹⁶ und R¹⁷ jeweils ein Wasserstoffatom oder ein Halogenatom bedeuten; R¹⁸ und R¹⁹ jeweils eine gegebenenfalls substituierte Alkylgruppe bedeuten; und Ar¹ eine gebenenfalls substituierte Arylengruppe bedeutet); (wobei R²⁰ eine gegebenenfalls substituierte Arylgruppe oder eine gegebenenfalls substituierte heterocyclische Gruppe bedeutet; R²¹ ein Wasserstoffatom, eine gegebenenfalls substituierte Alkylgruppe oder eine gegebenenfalls substituierte Arylgruppe bedeutet; Q ein Wasserstoffatom, ein Halogenatom, eine Alkylgruppe, eine substituierte Aminogruppe, eine Alkoxygruppe oder eine Cyangruppe bedeutet; und p eine ganze Zahl mit dem Wert 0 oder 1 ist); (wobei R²² eine gegebenenfalls substituierte Arylgruppe oder eine gegebenenfalls substituierte heterocyclische Gruppe bedeutet; R²³ ein Wasserstoffatom, eine gegebenenfalls substituierte Alkylgruppe oder eine gegebenenfalls substituierte Arylgruppe bedeutet; X'₂ ein Wasserstoffatom, ein Halogenatom, eine Alkylgruppe, eine substituierte Aminogruppe, eine Alkoxygruppe oder eine Cyangruppe bedeutet; und q eine ganze Zahl mit dem Wert 0 oder 1 ist); (wobei l eine ganze Zahl mit dem Wert 0 oder 1 ist; R²⁴, R²⁵ und R²⁶ jeweils eine gegebenenfalls substituierte Arylgruppe bedeuten; R²⁷ und R²⁸ jeweils ein Wasserstoffatom, eine Alkylgruppe mit 1 - 4 Kohlenstoffatomen, eine gegebenenfalls substituierte Aryl- oder Aralkylgruppe bedeuten, mit der Maßgabe, daß R²⁷ und R²⁸ nicht gleichzeitig ein Wasserstoffatom bedeuten, und daß für l = 0 R²⁷ nicht ein Wasserstoffatom bedeutet); (wobei R²⁹ und R³⁰ jeweils eine gegebenenfalls substituierte Alkyl- oder Phenylgruppe bedeuten, wobei der Substituent eine Alkyl-, Alkoxy- oder Phenylgruppe ist; R³¹ eine gegebenenfalls substituierte Phenyl-, Naphthyl-, Anthryl-, Fluorenylgruppe oder eine heterocyclische Gruppe bedeutet, wobei der Substituent eine Alkylgruppe, eine Alkoxygruppe, ein Halogenatom, eine Hydroxylgruppe oder eine Phenylgruppe ist; R³¹' ein Wasserstoffatom, eine gegebenenfalls substituierte Alkyl- oder Phenylgruppe bedeutet; und R³², R³³, R³⁴ und R³⁵ jeweils ein Wasserstoffatom, ein Halogenatom, eine Alkylgruppe, eine Alkoxygruppe oder eine Alkylaminogruppe bedeuten); (wobei Ar² und Ar³ jeweils eine gegebenenfalls substituierte Phenylgruppe bedeuten, wobei der Substituent ein Halogenatom, eine Alkylgruppe, eine Nitrogruppe oder eine Alkoxygruppe ist; und Ar⁴ eine gegebenenfalls substituierte Phenyl-, Naphthyl-, Anthryl-, Fluorenylgruppe oder heterocyclische Gruppe bedeutet, wobei es sich bei dem Substituenten um eine Alkylgruppe, eine Alkoxygruppe, ein Halogenatom, eine Hydroxylgruppe, eine Aryloxygruppe, eine Arylgruppe, eine Aminogruppe, eine Nitrogruppe, eine Piperidinogruppe, eine Morpholinogruppe, eine Naphthylgruppe, eine Anthrylgruppe oder eine substituierte Aminogruppe handelt, bei der der Substituent eine Acyl-, eine Alkyl-, eine Aryl- oder eine Aralkylgruppe ist; wobei D eine gegebenenfalls substituierte Phenylgruppe oder eine gegebenenfalls substituierte Carbazolylgruppe oder eine aus den Gruppen: ausgewählte Gruppe bedeutet, wobei R³⁶, R³⁷, R³⁸, R³⁹ und R⁴⁵ jeweils eine gegebenenfalls substituierte Alkylgruppe, eine gegebenenfalls substituierte Aralkylgruppe oder eine gegebenenfalls substituierte Arylgruppe darstellen; und R⁴⁰, R⁴¹, R⁴², R⁴³, R⁴⁴ und R⁴⁶ jeweils eine Alkylgruppe, eine Alkoxygruppe oder ein Halogenatom darstellen.

18. Photorezeptor gemäß Anspruch 1, in welchem es sich bei dem in der genannten Ladungsträgererzeugungsschicht enthaltenen Ladungsträgererzeugungsmaterial um ein polycyclisches Chinonpigment oder ein Bisazopigment handelt.

19. Photorezeptor gemäß Anspruch 16, in welchem es sich bei dem genannten polycyclischen Chinonpigment um ein durch die folgende allgemeine Formel (XI) dargestelltes Anthanthronpigment handelt: wobei X ein Halogenatom, eine Nitrogruppe, eine Cyangruppe, eine Acylgruppe oder eine Carboxylgruppe bedeutet; n eine ganze Zahl zwischen 0 und 4 ist; und m eine ganze Zahl zwischen 0 und 6 ist.

20. Photorezeptor gemäß Anspruch 16, in welchem es sich bei dem genannten Bisazopigment um ein durch die folgende allgemeine Formel (XVa) dargestelltes Fluorenylidenpigment handelt: wobei R⁵⁵ und R⁵⁶ jeweils eine Alkylgruppe, eine Alkoxygruppe oder eine Arylgruppe bedeuten; R⁵⁷, R⁵⁸, R⁵⁹, R⁶⁰, R⁶¹ und R⁶² jeweils ein Wasserstoffatom, ein Halogenatom, eine Alkylgruppe, eine Alkoxygruppe, eine Aminogruppe, eine Hydroxylgruppe oder eine Arylgruppe bedeuten; und A'' eine gegebenenfalls substituierte Arylgruppe bedeutet.

21. Photorezeptor gemäß Anspruch 16, in welchem es sich bei dem genannten Bisazopigment um ein durch die folgende allgemeine Formel (XVI) dargestelltes Fluorenonpigment handelt: wobei X¹ und X² jeweils ein Halogenatom, eine gegebenenfalls substituierte Alkylgruppe, eine gegebenenfalls substituierte Alkoxygruppe, eine Nitrogruppe, eine Cyangruppe, eine Hydroxylgruppe oder eine gegebenenfalls substituierte Aminogruppe bedeuten, mit der Maßgabe, daß wenigstens eines von X¹ und X² ein Halogenatom ist; p und q jeweils eine ganze Zahl mit den Werten 0,1 oder 2 darstellen, mit der Maßgabe, daß p und q nicht gleichzeitig null sind, und für p = 2 X¹ gleiche oder verschiedene Gruppen bedeuten kann, und daß für q = 2 X² gleiche oder verschiedene Gruppen bedeuten kann; und A eine durch die folgende allgemeine Formel (XVII) dargestellte Gruppe bedeutet: (wobei Ar⁸ eine aromatische carbocyclische oder heterocyclische Gruppe mit wenigstens einer fluorierten Kohlenwasserstoffgruppe bedeutet; Z die zur Bildung eines gegebenenfalls substituierten aromatischen Kohlenstoffrings oder eines gegebenenfalls substituierten aromatischen heterocyclischen Rings erforderlichen nichtmetallischen Atome darstellt); m und n jeweils eine ganze Zahl mit den Werten 0,1 oder 2 darstellen, mit der Maßgabe, daß m und n nicht gleichzeitig null sind.

22. Photorezeptor gemäß Anspruch 1, in welchem eine dem elektrisch leitfähigen Träger näher gelegene und der äußersten aufbauenden Schicht der genannten Ladungsträgertransportschicht benachbarte aufbauende Schicht der Ladungsträgertransportschicht ein Polycarbonat vom Typ Bisphenol A als Bindemittel enthält.

23. Photorezeptor gemäß Anspruch 1, in welchem das in einer dem elektrisch leitfähigen Träger näher gelegenen und der äußersten aufbauenden Schicht der genannten Ladungsträgertransportschicht benachbarten aufbauenden Schicht der genannten Ladungsträgertransportschicht enthaltene Bindemittelharz in dem bei der Beschichtung der genannten äußersten aufbauenden Schicht verwendeten Lösungsmittel kaum löslich ist.

24. Photorezeptor gemäß Anspruch 1, in welchem eine dem elektrisch leitfähigen Träger nächstgelegene aufbauende Schicht der genannten Ladungsträgertransportschicht durch Tauchbeschichtung und eine der genannten aufbauenden Schicht benachbarte und von dem elektrisch leitfähigen Träger entfernter liegende aufbauende Schicht der genannten Ladungsträgertransportschicht durch Sprühbeschichtung gebildet wird.

25. Photorezeptor gemäß Anspruch 1, in welchem eine dem leitfähigen Träger nächstgelegene aufbauende Schicht der genannten Ladungsträgertransportschicht eine Stärke von 5 - 50 µm aufweist.

26. Photorezeptor gemäß Anspruch 1, in welchem eine dem elektrisch leitfähigen Träger nächstgelegene aufbauende Schicht der genannten Ladungsträgertransportschicht eine Stärke von 5 - 30 µm aufweist.

27. Photorezeptor gemäß Anspruch 1, in welchem die äußerste aufbauende Schicht der genannten Ladungsträgertransportschicht eine Stärke von 0,1 - 30 µm aufweist.

28. Photorezeptor gemäß Anspruch 1, in welchem die äußerste aufbauende Schicht der genannten Ladungsträgertransportschicht eine Stärke von 0,5 - 10 µm aufweist.

29. Photorezeptor gemäß Anspruch 1, in welchem die genannte Ladungsträgererzeugungsschicht eine Stärke von 0,01 - 10 µm aufweist.

30. Photorezeptor gemäß Anspruch 1, in welchem die genannte Ladungsträgererzeugungsschicht eine Stärke von 1 - 5 µm aufweist.

## Revendications

1. Photorécepteur possédant une base électroconductrice, une couche engendrant un support formée par-dessus et une couche de transport du support étalée sur la couche engendrant un support et contenant une substance de transport du support et une substance liante; la couche de transport du support comprenant au moins deux couches constitutives de façon à ce que le rapport pondéral de la substance de transport du support à la substance liante dans une couche constitutive plus proche de la base électroconductrice soit plus élevé que le rapport pondéral de la substance de transport du support dans une couche constitutive plus éloignée de la base électroconductrice, et un polycarbonate possédant, comme motif récurrent principal, un motif structurel représenté par la formule (I) ou un motif structurel représenté par la formule (II), contenu dans la substance liante dans la couche constitutive la plus externe de la couche de transport du support: dans laquelle R¹ et R² sont chacun un atome d'hydrogène, un groupe aliphatique substitué ou non substitué, un groupe aromatique substitué ou non substitué; R³, R⁴, R⁵, R⁶, R⁷, R⁸, R⁹ et R¹⁰ sont chacun un atome d'hydrogène, un atome d'halogène, un groupe aliphatique substitué ou non substitué, un groupe carbocyclique substitué ou non substitué; dans laquelle Z est le groupe d'atomes nécessaire pour former un noyau carboné substitué ou non substitué ou un noyau hétérocyclique substitué ou non substitué; et l'un au moins des radicaux R¹ et R² est un des groupes (1) à (4) ci-dessous
(1) dans lequel R¹¹ est un atome d'hydrogène, un groupe alkyle ou un groupe ester alkylique représenté par -(CH₂)ₘCOOR, où R est un groupe alkyle, et m ≧ 1;
(2)
(3) un groupe alkyle représenté par -CₘH2ₘ₊₁, où m ≧ 4; et
(4) un groupe ester alkylique représenté par -(CH₂)ₘCOOR¹², où R¹² est un groupe alkyle, et m ≧ 2.

2. Photorécepteur selon la revendication 1, caractérisé en ce que le rapport de la substance de transport du support à la substance liante dans une couche constitutive la plus proche de la base électroconductrice est plus élevé que le rapport pondéral de la substance de transport du support à la substance liante dans la couche constitutive la plus externe de la couche de transport du support, la différence entre les deux rapport pondéraux étant d'au moins 20%.

3. Photorécepteur selon la revendication 2, caractérisé en ce que le rapport pondéral de la substance de transport du support à la substance liante dans une couche constitutive la plus proche de la base électroconductrice est plus élevé que le rapport pondéral de la substance de transport du support à la substance liante dans la couche constitutive la plus externe de la couche de transport du support, la différence entre les deux rapport pondéraux se situant dans l'intervalle de 20% à 140%.

4. Photorécepteur selon la revendication 1, caractérisé en ce que la couche de transport du support contient un polycarbonate possédant au moins un motif structurel représenté par la formule (II) comme motif récurrent principal.

5. Photorécepteur selon la revendication 1, caractérisé en ce que la couche constitutive la plus externe de la couche de transport du support renferme la substance de transport du support en une quantité d'au plus 70% en poids de la substance liante dans la couche constitutive la plus externe de la couche de transport du support.

6. Photorécepteur selon la revendication 5, caractérisé en ce que la couche constitutive la plus externe de la couche de transport du support renferme la substance de transport du support en une quantité de 5% à 70% en poids de la substance liante dans la couche constitutive la plus externe de la couche de transport du support.

7. Photorécepteur selon la revendication 1, caractérisé en ce que la couche constitutive de la couche de transport du support la plus proche de la base électroconductrice renferme la substance de transport du support en une quantité d'au plus 30% en poids de la substance liante dans la couche constitutive de la couche de transport du support la plus proche de la base électroconductrice.

8. Photorécepteur selon la revendication 7, caractérisé en ce que la couche constitutive de la couche de transport du support la plus proche de la base électroconductrice renferme la substance de transport du support en une quantité de 30% à 300% en poids de la substance liante dans la couche constitutive de la couche de transport du support la plus proche de la base électroconductrice.

9. Photorécepteur selon la revendication 1, caractérisé en ce que R¹ et R², dans la formule générale (I), représentent des groupes différents.

10. Photorécepteur selon la revendication 1, caractérisé en ce que l'un au moins des groupes R¹ et R², dans la formule générale (I), est un groupe volumineux comportant au moins 3 atomes de carbone.

11. Photorécepteur selon la revendication 1, caractérisé en ce que chacun des groupes R³ à R¹⁰, dans les formules générales (I) et (II), est un atome d'hydrogène, un atome d'halogène, un groupe méthyle ou un groupe cyclohexyle.

12. Photorécepteur selon la revendication 1, caractérisé en ce que Z, dans la formule générale (II), forme un noyau carboné ou un noyau hétérocyclique à 5 ou 6 chaînons.

13. Photorécepteur selon la revendication 1, caractérisé en ce que le nombre de répétitions du motif structurel représenté par les formules générales (I) ou (II) est de 10 à 5000.

14. Photorécepteur selon la revendication 13, caractérisé en ce que le nombre de répétitions du motif structurel représenté par les formules générales (I) ou (II) est de 50 à 2000.

15. Photorécepteur selon la revendication 1, caractérisé en ce que le polycarbonate posséde au moins un motif structurel représenté par la formule générale (II).

16. Photorécepteur selon la revendication 12, caractérisé en ce que les groupes R³ à R¹⁰, dans la formule générale (II), sont chacun un atome d'hydrogène et Z représente le groupe d'atomes nécessaire pour former un noyau cyclohexylidène.

17. Photorécepteur selon la revendication 1, caractérisé en ce que la substance de transport du support est l'un au moins des composés représentés par les formules générales (III) à (X) suivantes (dans laquelle R¹³ est un groupe aryle substitué ou non substitué; R¹⁴ est un atome d'hydrogène, un atome d'halogène, un groupe alkyle substitué ou non substitué, un groupe alcoxy, un groupe amino, un groupe hydroxyle ou un groupe amino substitué; et R¹⁵ est un groupe aryle substitué ou non substitué ou un groupe hétérocyclique substitué ou non substitué); (dans laquelle R¹⁶ et R¹⁷ sont chacun un atome d'hydrogène ou un atome d'halogéne; R¹⁸ et R¹⁹ sont chacun un groupe aryle substitué ou non substitué; et Ar¹ est un groupe arylène substitué ou non substitué); (dans laquelle R²⁰ est un groupe aryle substitué ou non substitué ou un groupe hétérocyclique substitué ou non substitué; R²¹ est un atome d'hydrogène, un groupe alkyle substitué ou non substitué ou un groupe aryle substitué ou non substitué; Q est un atome d'hydrogène, un atome d'halogène, un groupe alkyle, un groupe amino substitué, un groupe alcoxy ou un groupe cyano; et p est un nombre entier de 0 ou 1); (dans laquelle R²² est un groupe aryle substitué ou non substitué ou un groupe hétérocyclique substitué ou non substitué; R²³ est un atome d'hydrogène, un groupe alkyle substitué ou non substitué ou un groupe aryle substitué ou non substitué; X'₂ est un atome d'hydrogène, un atome d'halogène, un groupe alkyle, un groupe amino substitué, un groupe alcoxy ou un groupe cyano; et q est un nombre entier de 0 ou 1); (dans laquelle l est un nombre entier de 0 ou 1; R²⁴, R²⁵ et R²⁶ sont chacun un groupe aryle substitué ou non substitué; R²⁷ et R²⁸ sont chacun un atome d'hydrogène, un groupe alkyle comportant 1 à 4 atomes de carbone, un groupe aryle ou arylakyle substitué ou non substitué, à condition que R²⁷ et R²⁸ ne soient pas en même temps un atome d'hydrogène et que, lorsque l est nul, R²⁷ ne soit pas un atome d'hydrogène); (dans laquelle R²⁹ et R³⁰ sont chacun un groupe alkyle ou phényle substitué ou non substitué, le substituant étant un groupe alkyle, alcoxy ou phényle; R³¹ est un groupe phényle, naphtyle, anthryle, fluorényle ou un groupe hétérocyclique, substitué ou non substitué, le substituant étant un groupe alkyle, un groupe alcoxy, un atome d'halogène, un groupe hydroxyle ou un groupe phényle; R³¹, est un atome d'hydrogéne, un groupe alkyle ou phényle substitué ou non substitué; et R³², R³³, R³⁴ et R³⁵ sont chacun un atome d'hydrogène, un atome d'halogène, un groupe alkyle, un groupe alcoxy ou un groupe alkylamino); (dans laquelle Ar² et Ar³ sont chacun un groupe phényle substitué ou non substitué, le substituant étant un atome d'halogène, un groupe alkyle, un groupe nitro ou un groupe alcoxy; et Ar⁴ est un groupe phényle, naphtyle, anthryle, fluorényle ou hétérocyclique substitué ou non substitué, le substituant étant un groupe alkyle, un groupe alcoxy, un atome d'halogène, un groupe hydroxyle, un groupe aryloxy, un groupe aryle, un groupe amino, un groupe nitro, un groupe pipéridino, un groupe morpholino, un groupe naphtyle, un groupe anthryle ou un groupe amino substitué, dans lequel le substituant est un groupe acyle, un groupe alkyle, un groupe aryle ou un groupe arylalkyle); dans laquelle D est un groupe phényle substitué ou non substitué ou un groupe carbazolyle substitué ou non substitué, ou un groupe choisi dans les groupes dans lesquels R³⁶, R³⁷, R³⁸, R³⁹ et R⁴⁵ représentent chacun un groupe alkyle substitué ou non substitué, un groupe arylalkyle substitué ou non substitué ou un groupe aryle substitué ou non substitué; et R⁴⁰, R⁴¹, R⁴², R⁴³, R⁴⁴ et R⁴⁶ représentent chacun un groupe alkyle, un groupe alcoxy ou un atome d'halogène.

18. Photorécepteur selon la revendication 1, caractérisé en ce que la substance engendrant le support contenue dans ladite couche engendrant le support est un pigment quinone polycyclique ou un pigment bis-azoïque.

19. Photorécepteur selon la revendication 16, dans lequel ledit pigment quinone polycyclique est un pigment anthanthrone représenté par la formule générale (XI) suivante : dans laquelle X est un atome d'halogène, un groupe nitro, un groupe cyano, un groupe acyle ou un groupe carboxyle; n est un nombre entier de 0 à 4; et m est un nombre entier de 0 à 6.

20. Photorécepteur selon la revendication 16, dans lequel ledit pigment bis-azoïque est un pigment fluorénylidène représenté par la formule générale (XVa) suivante dans laquelle R⁵⁵ et R⁵⁶ sont chacun un groupe alkyle, un groupe alcoxy ou un groupe aryle; R⁵⁷, R⁵⁸, R⁵⁹, R⁶⁰, R⁶¹ et R⁶² sont chacun un atome d'hydrogène, un atome d'halogène, un groupe alkyle, un groupe alcoxy, un groupe amino, un groupe hydroxyle ou un groupe aryle; et A'' est un groupe aryle substitué ou non substitué.

21. Photorécepteur selon la revendication 16, dans lequel ledit pigment bis-azoïque est un pigment fluorénone représenté par la formule générale (XVI) suivante: dans laquelle X¹ et X² sont chacun un atome d'halogène, un groupe alkyle substitué ou non substitué, un groupe alcoxy substitué ou non substitué, un groupe nitro, un groupe cyano, un groupe hydroxyle ou un groupe amino substitué ou non substitué, à condition que l'un au moins des radicaux X¹ et X² soit un atome d'halogène; p et q représentent chacun un nombre entier de 0, 1 ou 2, à condition que p et q ne soient pas nuls en même temps et que, lorsque p est égal à 2, les radicaux X¹ puissent être des groupes identiques ou différents et que, lorsque q est égal à 2, les radicaux X² puissent être des groupes identiques ou différents; et A est un groupe représenté par la formule générale (XVII) suivante: (dans laquelle Ar⁸ est un groupe carbocyclique ou hétérocyclique aromatique possédant au moins un groupe hydrocarboné fluoré; Z représente les atomes non métalliques nécessaires pour former un noyau carboné aromatique substitué ou non substitué ou un noyau hétérocyclique aromatique substitué ou non substitué); m et n représentent chacun un nombre entier de 0, 1 ou 2, à condition que ni et n ne soient pas nuls en même temps.

22. Photorécepteur selon la revendication 1, dans lequel une couche constitutive de ladite couche de transport du support plus proche de la base électroconductrice et adjacente à la couche constitutive la plus externe de ladite couche de transport du support contient, comme liant, un polycarbonate de type bisphénol A.

23. Photorécepteur selon la revendication 1, dans lequel la résine liante contenue dans une couche constitutive de ladite couche de transport du support plus proche de la base électroconductrice et adjacente à la couche constitutive la plus externe de ladite couche de transport du support est très peu soluble dans le solvant utilisé pour revêtir ladite couche constitutive la plus externe.

24. Photorécepteur selon la revendication 1, dans lequel une couche constitutive de ladite couche de transport du support la plus proche de la base électroconductrice est formée par revêtement au trempé, et une couche constitutive de ladite couche de transport du support adjacente à ladite couche constitutive et éloignée de la base électroconductrice est formée par revêtement au pistolet.

25. Photorécepteur selon la revendication 1, dans lequel une couche constitutive de ladite couche de transport du support la plus proche de la base électroconductrice a une épaisseur de 5-50 µm.

26. Photorécepteur selon la revendication 1, dans lequel une couche constitutive de ladite couche de transport du support la plus proche de la base électroconductrice a une épaisseur de 5-30 µm.

27. Photorécepteur selon la revendication 1, dans lequel la couche constitutive la plus externe de ladite couche de transport du support a une épaisseur de 0,1-30 µm.

28. Photorécepteur selon la revendication 1, dans lequel la couche constitutive la plus externe de ladite couche de transport du support a une épaisseur de 0,5-10 µm.

29. Photorécepteur selon la revendication 1, dans lequel ladite couche engendrant le support a une épaisseur de 0,01-10 µm.

30. Photorécepteur selon la revendication 1, dans lequel ladite couche engendrant le support a une épaisseur de 0,1-5 µm.
